

# UNITED STATES PATENT OFFICE.

ALEXANDER WARFIELD, OF ALEXANDRIA, VIRGINIA.

## IMPROVED COMPOUND SOAP.

Specification forming part of Letters Patent No. 97,007, dated November 16, 1869.

*To all whom it may concern:*

Be it known that I, ALEXANDER WARFIELD, of Alexandria, in the county of Alexandria, and in the State of Virginia, have invented certain new and useful Improvements in Compound for Soap; and do hereby declare that the following is a full, clear, and exact description thereof.

The nature of my invention consists in a mixture or compound for soap which will save labor and expense.

In order to enable others skilled in the art to which my invention appertains to make and use the same, I will now proceed to describe the manner it is or may be mixed and used.

I take, first, ten pounds of olive or resin-soap, two quarts of lye strong enough to float an egg, two ounces pearl-ash of commerce, and two ounces of borax. These ingredients are mixed thoroughly, the soap being first shaved fine, and boiled until the soap is entirely dissolved. When cool I add eight ounces spirits of turpentine, eight ounces benzine, and eight ounces aqua ammonia, F F F F. If any perfume is desired it may be added at the same time as the above three ingredients. The whole compound is then mixed thoroughly and put in a vessel, or made into bars, cakes, or other convenient form.

Take four tubs of cold water—four gallons in the first tub, six in the second, and about ten in each of the other two. Add half a pound of my soap to the first tub and let the clothes remain from three to five minutes in the same, when they are to be wrung out. (No rubbing required,

unless very dirty, when they may be rubbed lightly.) The clothes are then put in the second tub and rinsed out, and in like manner in the third and fourth tubs, when they are put on the line in a perfectly-white condition—no bluing required.

The water in the first tub is replenished from the second tub when more clothes are to be washed, and one ounce of soap is added about every half hour to keep up the action of the clothes.

Clothes that fade badly can be washed without injury by adding one-fourth of an ounce of alum.

This soap is very cheap, and, as no rubbing or boiling is required, it saves both labor and expense.

I do not confine myself to the exact proportions of the ingredients above mentioned, as they may be varied slightly without materially changing the nature or the action of the soap.

Having thus fully described my invention, what I claim as new, and desire to secure by Letters Patent, is—

The compound for soap above described, when made substantially of the ingredients and in the manner herein set forth.

In testimony that I claim the foregoing I have hereunto set my hand this 1st day of November, 1869.

ALEXR. WARFIELD.

Witnesses:

J. M. MASON,  
A. N. MARR.